

3,192,159

## WATER-IN-OIL EMULSION LUBRICANT AND HYDRAULIC FLUID

Charles E. Francis, Martinez, Calif., assignor to Shell Oil Company, New York, N.Y., a corporation of Delaware  
No Drawing. Filed Oct. 17, 1961, Ser. No. 145,766  
11 Claims. (Cl. 252—33.6)

This invention relates to improved fire-resistant hydraulic fluids. More particularly, it pertains to water-in-oil colliery hydraulic fluids and lubricants which are fire and wear-resistant, stable and non-corrosive and to oil concentrates which are readily emulsifiable with large amounts of water.

Although it is known in the art that certain emulsions are useful as coolants and lubricants in metal working operations, the use of emulsions in hydraulic systems has been limited because of their inability to resist wear, their poor stability and their inability to pass fire-resistant requirements for which such fluids are primarily used.

In colliery equipment such as various hydraulic machinery, e.g., winder brake mechanism and wagon tipper to hydraulic jacks, pit props and roof bar straighteners, mechanical loaders and various other fluid drive mechanisms which are subject to load, shock and vibration, it is essential that the hydraulic fluid employed therein function properly and efficiently without the danger of being flammable or toxic.

A variety of so-called fire-resistant fluids are commercially available such as phosphate ester base fluids, but these have been found to possess poor low temperature viscosity-temperature properties, and they are toxic. Water-glycol solution or various water-oil emulsions have been found to have a tendency to form deposits and cause wear under high pressures and are costly.

It is an object of this invention to provide a composition which can be emulsified readily on the job to yield a fire resistant hydraulic fluid having good lubricating properties. Another object is to provide a fluid which after emulsification is a satisfactory lubricant for colliery hydraulic equipment, which is stable, non-toxic, fire-resistant to deterioration, inhibits corrosion and not cause wear. Still another object of this invention is to provide a water-mineral oil emulsion usable as lubricants and fire-resistant hydraulic fluids for various equipment used in colliery hydraulic equipment.

These and other objects are accomplished in accordance with this invention by providing a highly aromatic high viscosity index mineral oil base concentrate which is readily emulsifiable with a large amount of water, and which contains two particular types of dissimilar non-ionic surface active agents and an alkali metal dithiocarbamate or a mixture of alkali metal dithiocarbamate and alkali metal mercaptobenzothiazole, the metal portion being selected from the group consisting of sodium and potassium, all of the additives being present in critical amounts. Oil concentrates of this invention are readily emulsified with large amounts of water (20—45%) to form a stable, fire-resistant water-in-oil emulsion, particularly useful in colliery hydraulic equipment. If desired small amounts of polyvalent metal dithiocarbamates, the metal portion of the compound being selected from the group consisting of zinc, cadmium and/or lead and an alkylene glycol or ether derivative thereof can be added to the oil concentrate to improve emulsification and cold storage stability of the finished water-in-oil emulsion.

The highly aromatic mineral oil base should be one having a viscosity index (Dean Davis) of at least 80, preferably between 90 and 100. Mineral oil fraction should also be in the lubricating oil range and have a viscosity, as determined at 100° F., of from 75 to 250

SUS, preferably between 100 and 150 and an aromatic content of from about 10% to about 30%.

A typical mineral oil base is a high viscosity index highly solvent refined mineral lubricating oil having the following properties.

|    |                               |       |
|----|-------------------------------|-------|
| 5  | Gr. ° API, 60° C.             | 32.2  |
|    | Color, ASTM                   | 1     |
|    | Pour point, ° F.              | 5     |
|    | Flash, ° F., COC              | 370   |
| 10 | Fire, ° F.                    | 435   |
|    | Viscosity, SUS at 100° F.     | 103   |
|    | Viscosity index               | 93    |
| 15 | Neutralization No.            | 0.01  |
|    | Components, percent w.t.      |       |
|    | n-Alkanes                     | 21.8  |
|    | Isoalkenes                    | 11.8  |
|    | Noncondensed cycloalkanes     | 24.9  |
| 20 | Condensed cycloalkanes        | 12.4  |
|    | Total saturates               | 70.9  |
|    | Monoaromatics                 | 13.6  |
|    | Diaromatics                   | 5.8   |
| 25 | Triaromatics                  | 4.0   |
|    | Tetraaromatics                | 1.6   |
|    | Pentaaromatics                | 0.2   |
|    | Hexaaromatics                 |       |
|    | Total sulfur compounds        | 3.9   |
|    | Total                         | 100.0 |
| 30 | Sulfur analysis, percent w.t. |       |
|    | Thiopenes                     |       |
|    | Benzo-                        | 1.7   |
|    | Triaromatics                  | 0.5   |
|    | Tetraaromatics                | 0.4   |
| 35 | Pentaaromatics                |       |
|    | Other sulfur compounds        | 1.3   |
|    | Total                         | 3.9   |

The two non-ionic surface agents and the metal compounds defined above may be added to the mineral oil and these compounds are (1) a monoester of a long chain fatty acid having at least 8 carbon atoms and an inner ether of aliphatic polyhydric alcohols such as hexahydric alcohols and (2) a polyalkylenoxy phenoxy alkanol, and (3) an alkali metal dithiocarbamate or a mixture of (a) alkali metal thiocarbamate and (b) alkali metal mercaptobenzothiazole. Each of these additives must be present in critical amounts of which the monoester (1) be used in amounts ranging from 1% to 4%, preferably from 1.5% to 3% and the polyalkylenoxy phenoxy alkanol (2) is used in amounts ranging from 0.5% to 3%, preferably from 1% to 2%, and (3) is used in amounts of from 0.01% to 1.0%, each by weight.

In the monoester non-ionic surface agent the inner ether alcohol is prepared by partially dehydrating polyhydric alcohols which results in the conversion of the polyhydric alcohol to inner ether polyhydric compounds having 1 or 2 ethers and 4 to 6 hydroxyl groups in the molecule in the manner described in U.S. Patent 2,322,820. Compounds of this type are exemplified by sorbitan, mannan, xylitan, dulcitan, etc. Fatty acids which are used to form the monoesters of the inner ether polyalcohols are saturated and unsaturated fatty acids having at least 8 carbon atoms, preferably from 12 to 18 carbon atoms, such as lauric, stearic, oleic, linoleic, ricinoleic acids and the like. Monoesters of this type include sorbitan monolaurate, sorbitan monostearate, sorbitan monooleate, sorbitan monoricinoleate, mannan monolaurate, mannan monooleate, and mixtures thereof. Compounds of this type are available commercially as "Span 20, 60, or 80" from the Atlas Powder Company. The second essential additive is an oil-soluble alkyl

phenoxy polyalkylene glycol having the formula R-phenyl (—OR')—<sub>n</sub>OR''—OH, wherein n is an integer of from 2 to 6, preferably 3 to 4, R is an alkyl radical of 4 to 20 carbon atoms, preferably 4 to 12, and R' and R'' are the same or different alkylene groups such as ethylene or propylene groups, they are preferably the same, and preferably ethylene. Compounds of this type are C<sub>4-12</sub> alkyl phenoxy(alkoxy)<sub>4-6</sub> alkanols exemplified by isobutylphenoxy tetraethyleneoxy ethanol, diisobutylphenoxy tetraethyleneoxy ethanol, nonylphenoxy tetraethyleneoxy ethanol, octylphenoxy hexaethyleneoxy ethanol, diisobutylphenoxy tripropyleneoxy propanol, and mixtures thereof.

The third component as defined is used in amounts of from about 0.01% to about 1%. When mixtures are used the proportions of the mixture may vary from 10% to 90% (25-75%) of alkali metal dithiocarbamate and 90% to 10% (75-25%) of alkali metal mercaptobenzothiazole. The general formula of the alkali metal dithiocarbamate is



wherein M is sodium or potassium, R<sub>1</sub> is a hydrocarbyl radical such as alkyl, aralkyl, alkaryl, cycloalkyl; R<sub>2</sub> can be the same or different hydrocarbyl radical from R<sub>1</sub> or it can be hydrogen; it is desirable that both R radicals are alkyl radicals from 1 to 16 carbon atoms in which the alkyl radicals can be of same different chain length and structure, and it is preferred that the R's are C<sub>1-12</sub> alkyl radicals of the same chain length but different structure. Examples of such salts are sodium and/or potassium dimethyl, dibutyl, diethyl, dihexyl, diisobutyl, dioctyl, dicyclohexyl, dicresyl, dithiocarbamates of which the preferred are sodium dimethyl dithiocarbamate, sodium dibutyl dithiocarbamate, sodium diisobutyl dithiocarbamate and sodium diethyl dithiocarbamate.

The other portion of mixture (3) includes sodium or potassium mercaptobenzothiazole. Preferred mixture of (3) includes 90-10 mixtures of sodium methyl dithiocarbamate and sodium mercaptobenzothiazole, sodium dibutyl dithiocarbamate and sodium mercaptobenzothiazole, sodium diaryl dithiocarbamate and sodium mercaptobenzothiazole, sodium diisobutyl dithiocarbamate and sodium mercaptobenzothiazole, potassium dibutyl dithiocarbamate and potassium mercaptobenzothiazole, and potassium diethyl dithiocarbamate and potassium mercaptobenzothiazole.

In addition to the above essential additives, stability and emulsifiability can be improved by addition of small amounts (0.01-0.5% each) of polyvalent metal dithiocarbamate and alkylene glycol or its ether derivatives.

The polyvalent metal dithiocarbamates includes the zinc, cadmium or lead salts of N- or N,N'-C<sub>1-8</sub> alkyl substituted dithiocarbamic acid such as zinc, cadmium, or lead dipropyl mono and dithiocarbamate, dibutyl mono and dithiocarbamate, diethyl mono and dithiocarbamate, dihexyl mono and dithiocarbamate, dioctyl mono and dithiocarbamate, di-2-ethylhexyl mono and dithiocarbamate, di-isobutylmono and dithio-carbamate, diisooamyl dithiocarbamate mono and N-amyl-N'-methyl mono and dithiocarbamate, N-methyl-N'-octyl mono and dithiocarbamate, N-octyl-N'-butyl mono and dithiocarbamate, N-n-amyl-N'-2-methylbutyl dithiocarbamate, N-n-amyl-N'-3-methylbutyl dithiocarbamate, N-octyl-N'-2-ethylhexyl dithiocarbamate, N-ethyl-N'-phenyl mono and dithiocarbamate, dicyclohexyl mono and dithiocarbamate, diphenyl mono and dithiocarbamate, and the like.

The alkylene glycols and the ether derivatives thereof includes ethylene glycol, diethylene glycol, triethylene glycol, tetraethylene glycol, propylene glycol, dipropylene glycol, hexylene glycol and mixtures thereof.

In addition to the above essential additives it is preferred to use in such compositions small amounts of from about 0.01% to about 2%, preferably from about 0.2% to

75 about 1% of oil soluble antioxidants. The antioxidants include phenolic and aromatic soluble antioxidants. The antioxidants includes phenolic and aromatic amine compounds. The phenolic compounds are illustrated by the alkyl phenols, e.g., di- and trialkyl phenols, for instance 2,4-, 2,3-, 3,4-, 2,6- and 3,5-diamyl phenol, 2,4-dimethyl-6-tert. butylphenol, 2,6-ditert.butyl-4-methylphenol, as well as bisphenols such as 4,4'methylene-bis(2,6-ditert. butylphenol). The amines are illustrated by arylamines such as phenyl-alpha-naphthylamine or phenyl-beta-naphthylamine.

Illustrative examples of mineral oil bases of this invention which are emulsified with from about 20% to about 45%, preferably from about 30% to about 40% of water to form a stable fire-resistant hydraulic fluid are presented below.

Percent wt.

Composition A:

|  |                                                                              |         |
|--|------------------------------------------------------------------------------|---------|
|  | Sorbitan mono-oleate                                                         | 2       |
|  | Diisobutylphenoxy(ethoxy) <sub>4</sub> ethanol                               | 1       |
|  | Sodium dimethyl dithiocarbamate—sodium mercaptobenzothiazole, 90/10% mixture | 0.5     |
|  | Mineral lubricating oil (X)                                                  | Balance |

Composition B:

|  |                                                                          |         |
|--|--------------------------------------------------------------------------|---------|
|  | Sorbitan mono-oleate                                                     | 2       |
|  | Diisobutylphenoxy(ethoxy) <sub>4</sub> ethanol                           | 1       |
|  | Sodium dibutyl dithiocarbamate—sodium mercaptobenzothiazole, 50% mixture | 0.5     |
|  | Mineral lubricating oil (X)                                              | Balance |

Composition C:

|  |                                                                          |         |
|--|--------------------------------------------------------------------------|---------|
|  | Sorbitan mono-oleate                                                     | 2       |
|  | Diisobutylphenoxy(ethoxy) <sub>4</sub> ethanol                           | 1       |
|  | Sodium diethyl dithiocarbamate—sodium mercaptobenzothiazole, 50% mixture | 0.5     |
|  | Mineral lubricating oil (X)                                              | Balance |

Composition D:

|  |                                                |         |
|--|------------------------------------------------|---------|
|  | Sorbitan mono-oleate                           | 2       |
|  | Diisobutylphenoxy(ethoxy) <sub>4</sub> ethanol | 1       |
|  | Sodium dimethyl dithiocarbamate                | 0.01    |
|  | 2,6-ditert.butyl-4-methyl phenol               | 0.2     |
|  | Phenyl-alpha-naphthylamine                     | 0.1     |
|  | Mineral lubricating oil (X)                    | Balance |

Composition E:

|  |                                                                              |         |
|--|------------------------------------------------------------------------------|---------|
|  | Mannitan mono-oleate                                                         | 2       |
|  | Diisobutyl-phenoxy(ethoxy) <sub>6</sub> ethanol                              | 1       |
|  | Sodium dimethyl dithiocarbamate—sodium mercaptobenzothiazole, 90/10% mixture | 0.5     |
|  | 2,6-ditert.butyl-4-methyl phenol                                             | 0.2     |
|  | Phenyl-alpha-naphthylamine                                                   | 0.1     |
|  | Mineral lubricating oil (X)                                                  | Balance |

Composition F:

|  |                                                                              |         |
|--|------------------------------------------------------------------------------|---------|
|  | Mannitan mono-oleate                                                         | 2       |
|  | Nonylphenoxy(ethoxy) <sub>4</sub> ethanol                                    | 1       |
|  | Sodium dimethyl dithiocarbamate—sodium mercaptobenzothiazole, 90/10% mixture | 0.5     |
|  | 4,4'-methylene (2,6-ditert.butylphenol)                                      | 0.2     |
|  | Phenyl-alpha-naphthylamine                                                   | 0.1     |
|  | Mineral lubricating oil (X)                                                  | Balance |

Composition G:

|  |                                                                           |         |
|--|---------------------------------------------------------------------------|---------|
|  | Sorbitan mono-oleate                                                      | 2       |
|  | Diisobutylphenoxy(ethoxy) <sub>4</sub> ethanol                            | 1       |
|  | Sodium dimethyl dithiocarbamate—sodium mercaptobenzothiazole, 50% mixture | 0.5     |
|  | 2,6-ditert.butyl-4-methyl phenol                                          | 0.2     |
|  | Phenyl-alpha-naphthylamine                                                | 0.1     |
|  | Cadmium diethyl dithiocarbamate                                           | 0.025   |
|  | Mineral lubricating oil (X)                                               | Balance |

Composition H:

|  |                                                |         |
|--|------------------------------------------------|---------|
|  | Sorbitan mono-oleate                           | 2       |
|  | Diisobutylphenoxy(ethoxy) <sub>8</sub> ethanol | 1       |
|  | Sodium dimethyl dithiocarbamate                | 0.01    |
|  | 2,6-ditert.butyl-4-methyl phenol               | 0.2     |
|  | Phenyl-alpha-naphthylamine                     | 0.1     |
|  | Zinc diethyl dithiocarbamate                   | 0.025   |
|  | Ethylene glycol                                | 0.2     |
|  | Mineral lubricating oil (X)                    | Balance |

The finished emulsion fluid is prepared by slowly adding to the oil base composition such as A, B, C, D, E, F, G or H from 20% to 45% based on the total composition, an aqueous base, such as water which may or may not contain 0.1% to 1% of a corrosion or wear inhibitor such as water-soluble inorganic nitrites, nitrates, chromates, phosphates or water-soluble low molecular weight salts such as alkali metal or alkaline earth metal (Na, K, Ca, Ba) acetate or propionate. The water-in-oil emulsion can be mixed by any suitable means such as by air agitation, propeller agitation or by passing through a colloid mill until a homogeneous stable water-in-oil emulsion is formed. For economical reasons, the water is added to the oil in desired amounts at the time the emulsion is to be used, although a stable water-in-oil emulsion can be prepared and stored for a moderate period.

A finished water-in-oil emulsion (Composition I) was prepared by admixing 60% of composition D with 40% water and the mixture was passed through a colloid mill until a stable homogeneous water-in-oil emulsion was formed.

Other finished compositions include:

|                                         | Percent |
|-----------------------------------------|---------|
| Composition II—                         |         |
| Water                                   | 30      |
| Composition A                           | 70      |
| Composition III—                        |         |
| Water containing 0.1% Ca acetate        | 40      |
| Composition G                           | 60      |
| Composition IV—                         |         |
| Water containing 0.1% NaNO <sub>2</sub> | 35      |
| Composition C                           | 65      |
| Composition V—                          |         |
| Water                                   | 40      |
| Composition H                           | 60      |

The outstanding emulsion stability properties of these compositions is demonstrated by compositions I and V in Table 1 in comparison with composition W\* which does not contain a metal carbamate. The stability was determined by measuring the amount of oil and water separation at 140° F. from a 100 ml. sample. Also in a Vicker's Hydraulic Pump Test similar to that described in "Lubrication Engineering," February 1949, pages 16-17, negligible wear was noted using compositions I and V after 1000 hours' testing, whereas compositions X\* and Y\* resulted in phase separation in from about 1 to 2 days.

Table 1

| Composition                   | I   |       | V      |       | W     |        |
|-------------------------------|-----|-------|--------|-------|-------|--------|
|                               | Oil | Water | Oil    | Water | Oil   | Water  |
| Emulsion Stability at 140° F. |     |       |        |       |       |        |
| Separation, percent           |     |       |        |       |       |        |
| V.:                           |     |       |        |       |       |        |
| 1 day                         | 1   | <1    | Slight | Trace | 1     | Slight |
| 10 days                       | 1   | 1     | 2      | <1    | 15    | Slight |
| 20 days                       | 5   | 1     | 6      | <1    | 37    | Slight |
| 25 days                       | 9   | 1     | 8      | <1    | 45    | 2      |
| 30 days                       | 13  | 1     | 12     | <1    | ----- | -----  |
| 40 days                       | 22  | 2     | 24     | <1    | ----- | -----  |

Compositions of the present invention such as compositions I through V are fire-resistant passing over 50 cycles as determined by the Pipe Cleaner Test described in Lubricating Engineering, March-April 1955, pages 86-87 while a neat mineral oil or a mineral oil containing 4%

\*Composition W: [water-in-oil emulsion comprising 40% water plus 60% mineral oil composition containing 2% sorbitan monooleate (Span 80)+1% diisobutylphenoxy(ethoxy) ethanol+0.2% 2,6-ditertiarybutyl-4-methyl phenol+0.1% phenyl alaphenylthylamine].

\*Composition X: [water-in-oil emulsion comprising 40% water+60% mineral oil composition containing +5% polyethylene substituted sorbitan monooleate (Tween 81)+0.15% glycerol monooleate+0.12% sulfurized oleic acid].

\*Composition Y: [oil-in-water emulsion comprising 50% water+50% mineral oil composition containing 20% Na petroleum sulfonate, 1% ricinoleic acid, 1% hexylene glycol, 1% lard oil, 2% water, 0.3% Dowicide O, 0.1% sodium hydroxide and the balance mineral oil].

each of Ca petroleum sulfonate and/or Ca C<sub>12-22</sub> alkyl salicylate ignited after 5 cycles.

I claim as my invention:

1. A water-in-oil emulsion lubricant and hydraulic fluid which is from about 20% to about 45% water phase and from about 55% to about 80% oil phase, the oil phase being essentially a 80-100 VI mineral oil having a viscosity in the range of from 75 to 250 SUS at 100° F. containing (1) from about 1% to about 4% of a monoester of a long chain fatty acid having from 8 to 18 carbon atoms and an inner ether of an aliphatic polyhydric alcohol having 1-2 ether and 4-6 hydroxyl groups, (2) from about 0.5% to about 3% of an oil-soluble C<sub>4-20</sub> alkyl phenoxy(C<sub>2-3</sub> alkyl oxy)<sub>4-6</sub> C<sub>2-3</sub> alkanol, and (3) from about 0.01% to about 1% of a material selected from the group consisting of alkali metal C<sub>1-12</sub> alkyl substituted dithiocarbamate and a mixture of 10-90% of an alkali metal C<sub>1-12</sub> alkyl substituted dithiocarbamate and 90-10% alkali metal mercaptobenzothiazole.
2. A water-in-oil emulsion lubricant and hydraulic fluid which is from about 20% to about 45% water phase and from about 55% to about 80% oil phase, the oil phase being essentially a 80-100 VI mineral oil having a viscosity in the range of from 75 to 250 SUS at 100° F. containing (1) from about 1.5% to about 3% of a monoester of a fatty acid having from 12 to 18 carbon atoms and an inner ether of an aliphatic hexahydric alcohol having 1-2 ether and 4-6 hydroxyl groups, (2) from about 1% to about 2% of an oil-soluble C<sub>4-12</sub> alkyl phenoxy(ethoxy)<sub>4-6</sub> ethanol, and (3) from about 0.01% to about 1% of a material selected from the group consisting of an alkali metal C<sub>1-12</sub> alkyl substituted dithiocarbamate and a mixture of 25-75% of an alkali metal C<sub>1-12</sub> alkyl substituted dithiocarbamate and 75-25% of an alkali metal mercaptobenzothiazole.
3. A water-in-oil emulsion lubricant and hydraulic fluid which is from about 20% to about 45% water phase and from about 55% to about 80% oil phase, the oil phase being essentially a 80-100 VI mineral lubricating oil having a viscosity in the range of from 100 to 150 SUS at 100° F. containing from about 1.5% to about 3% of a sorbitan monooleate, from about 1% to about 2% of an alkyl mixture of phenoxy(ethoxy)<sub>4-6</sub> ethanol and from about 0.01% to about 1% of a mixture of 10-90% of sodium dimethyl dithiocarbamate and 90-10% of sodium mercaptobenzothiazole.
4. The composition of claim 2 containing in the emulsion from 0.01% to 2% of an oil-soluble antioxidant selected from the group consisting of alkyl substituted simple phenol and phenyl-alpha-naphthylamine and mixtures thereof.
5. The composition of claim 2 containing in the emulsion from about 0.01% to about 1% of an oil-soluble polyvalent metal N,N'-C<sub>1-8</sub> alkyl substituted dithiocarbamate, the metal being selected from the group consisting of zinc, cadmium and lead.
6. The composition of claim 3 containing in the emulsion from 0.01% to 2% of an oil-soluble antioxidant selected from the group consisting of alkyl substituted simple phenol and phenyl-alpha-naphthylamine and mixtures thereof.
7. The composition of claim 3 containing in the emulsion from about 0.01% to about 1% of an oil-soluble polyvalent metal N,N'-C<sub>1-8</sub> alkyl substituted dithiocarbamate, the metal being selected from the group consisting of zinc, cadmium and lead.
8. A water-in-oil emulsion lubricant and hydraulic fluid which is from about 30% to about 40% water phase and from about 70% to about 60% oil phase, the oil phase being essentially a 80-100 VI mineral lubricating oil containing from about 1.5% to about 3% of sorbitan monooleate, from about 1% to about 2% of an oil-soluble diisobutylphenoxy(ethoxy)<sub>4</sub> ethanol and from about 0.01% to about 1% of a 50-50 mixture of sodium dimethyl dithiocarbamate and sodium mercaptobenzothiazole.

9. The composition of claim 8 containing in the emulsion from about 0.01% to about 1% each of an oil-soluble alkylphenol, an oil-soluble arylamine and polyvalent metal N,N'-C<sub>1-8</sub> alkyl substituted dithiocarbamate, the metal being selected from the group consisting of zinc, cadmium and lead. 5

10. The composition of claim 8 containing in the emulsion from about 0.01% to about 1% each of 2,6-ditert-butyl-4-methylphenol, phenyl-alpha-naphthylamine and zinc diamylidithiocarbamate.

11. The composition of claim 8 containing in the emulsion from about 0.01% to about 1% each of 2,6-ditert-

butyl-4-methylphenol, phenyl-alpha-naphthylamine and ethylene glycol.

**References Cited by the Examiner**

**UNITED STATES PATENTS**

|           |       |            |          |
|-----------|-------|------------|----------|
| 2,625,509 | 1/53  | Lang       | 252—49.5 |
| 2,681,891 | 6/54  | Bos et al. | 252—75   |
| 3,003,957 | 10/61 | Barkis     | 252—49.5 |
| 3,050,465 | 8/62  | Francis    | 252—77 X |

JULIUS GREENWALD, *Primary Examiner.*

JOSEPH R. LIBERMAN, ALBERT T. MEYERS,  
*Examiners.*